

[54] NON-CATALYTIC DURABLE PRESS  
PROCESS FOR TREATING CELLULOSIC  
MATERIAL USING FORMALDEHYDE  
VAPOR AND POST-HEATING

[75] Inventors: Jose P. Gamarra, San Jose; Ronald Swidler, Palo Alto, both of Calif.

[73] Assignee: Cotton, Incorporated, New York, N.Y.

[22] Filed: July 13, 1972

[21] Appl. No.: 271,237

[52] U.S. Cl..... 8/182, 2/243, 8/115.7,  
8/129, 8/149.2, 8/182, 8/184, 8/185, 8/186,  
8/187, 8/189, 8/194, 8/DIG. 4, 8/DIG. 9,  
8/DIG. 10, 8/DIG. 21, 28/144

[51] Int. Cl... D06m 13/14, D06m 13/40, D06m 13/54

[58] Field of Search ..... 38/144; 2/243; 8/116.4,  
8/182, 184, 185, 186, 187, 189, 194

## [56] References Cited

## UNITED STATES PATENTS

3,545,913 12/1970 Joarder et al..... 8/116.4  
3,653,805 4/1972 Gamarra et al..... 8/116.3  
3,663,158 5/1972 Brenner et al..... 8/116.4

## OTHER PUBLICATIONS

Joarder et al., Textile Research Journal 37,  
1083-1084 (1967).  
Joarder et al., Textile Research Journal, 39, 49-54  
(1969).

Chemical Abstracts, 58, 9268g.

Gagliardi et al., Textile Research Journal, 36,  
168-177 (1966).Mehta et al., Journal of the Textile Institute, 58,  
279-292 (1967).

Primary Examiner—George F. Lesmes

Assistant Examiner—J. Cannon

Attorney, Agent, or Firm—Burns, Doane, Swecker &  
Mathis

## [57] ABSTRACT

The dimensional stability, wrinkle resistance, smooth drying characteristics and total shape retentivity of cellulosic material such as cotton fabrics are improved by impregnating the fabric with an aqueous solution of a monomeric compound which has at least one active hydrogen and reacts with formaldehyde, e.g., urea, exposing the impregnated fabric to an atmosphere containing formaldehyde vapors in the absence of a catalyst until a creaseproofing amount of an at least partially polymerized, substantially water-insoluble condensate (such as an amide-formaldehyde condensate) is affixed to the fabric without, however, effecting any substantial amount of cross-linking with the cellulosic fiber. The thus-exposed fabric is thereafter post-heated in an inert gaseous atmosphere also in the absence of a catalyst to further polymerize and cross-link the fabric.

9 Claims, No Drawings

**NON-CATALYTIC DURABLE PRESS PROCESS  
FOR TREATING CELLULOSIC MATERIAL USING  
FORMALDEHYDE VAPOR AND POST-HEATING**

**BACKGROUND OF THE INVENTION**

In recent years, various methods have been devised for treating cellulosic fiber-containing products such as cloth made of cotton or cotton blends in order to impart durable wrinkle resistance and smooth drying characteristics thereto. For example, cellulosic materials have been cross-linked with formaldehyde in the presence of a number of various catalysts giving durable cross-links having good resistance to repeated laundering and also to various acids and alkalies and chlorine bleaches.

U.S. Pat. No. 3,653,805, for example, discloses impregnating the cellulosic material with a formaldehyde-reactive compound, such as urea and then contacting the impregnated fabric with formaldehyde vapors to form an insoluble reaction product on the fabric in the absence of an acidic catalyst and without effecting sufficient cross-linking with the cellulosic fiber to produce an increase in wrinkle recovery high enough to interfere with subsequent shaping of the formaldehyde polymer-containing fabric. The fabric is thereafter impregnated with a latent solid acid catalyst or exposed to a gaseous catalyst and cured to give a durable press product.

Indeed, many of the prior art processes relating to durable press products using formaldehyde or formaldehyde-reactive materials have involved the use of acidic catalysts such as sulfur dioxide, formic acid, acetic acid, zinc chloride and the like. While these catalysts are effective in causing cross-linking or curing of the materials, they may degrade the physical properties of the cellulosic material.

The use of an uncatalyzed method for producing a durable press product has been attempted in the prior art, but no commercially suitable process has heretofore been found insofar as extremely long reaction times, e.g., 10 hours, were required to even approach acceptable minimum durable press property levels. See, for example, "An Uncatalyzed, Vapor-Phase Cross-linking Reaction of Cotton Cellulose with Formaldehyde," Joarder et al., Textile Research Journal, 39, No. 1, pp. 49-54 (January, 1969).

Therefore, the search has continued for a relatively rapid non-catalytic process able to give rise to an improved balance between physical properties and durable press properties for cellulosic materials such as cotton fabric.

**SUMMARY OF THE INVENTION**

Accordingly, a primary object of the present invention is to provide a non-catalytic durable press process for treating fiber-containing cellulosic materials which process substantially prevents or alleviates the problems mentioned above.

A more specific object is to provide a non-catalytic process which imparts an improved balance of durable press and physical properties to cellulosic materials.

Another specific object is to provide a non-catalytic durable press process for use with cellulosic materials which produces improved wrinkle resistance and smooth drying characteristics, keeps any loss of tensile

strength and abrasion resistance to a minimum, and requires relatively short processing time.

These and other objects, as well as the scope, nature and utilization of the invention will become more clearly apparent from the following more detailed description. Unless otherwise indicated, all proportions and percentages of materials or compounds are expressed on a weight basis throughout this specification and appended claims.

10 in accordance with the present invention, a non-catalytic process is provided for improving the dimensional stability, wrinkle resistance, smooth-drying characteristics and total shape retentivity of a cellulosic fiber-containing fabric which comprises: (a) applying to the cellulosic fiber-containing fabric a catalyst-free aqueous solution of a monomeric compound which has at least one active hydrogen and reacts with formaldehyde; (b) exposing the impregnated fabric to an atmosphere containing formaldehyde vapors in the absence of a catalyst until a creaseproofing amount of an at least partially polymerized condensate of the monomeric compound and formaldehyde in substantially water-insoluble form is affixed on said fabric without effecting any substantial amount of cross-linking with the cellulosic fiber; and (c) post-heating said fabric in an inert gaseous atmosphere in the absence of a catalyst at a temperature of from about 100° C. to about 180° C. for from about 1 to about 20 minutes to further polymerize and cross-link the fabric.

30 The essence of the present invention is the discovery that by post-heating in the absence of a catalyst or formaldehyde a fabric which has been impregnated with a catalyst-free aqueous solution of a monomeric compound which has at least one active hydrogen and reacts with formaldehyde, such as urea, and then exposed to formaldehyde vapors (again in the absence of a catalyst), a substantially improved wrinkle resistance and a significantly reduced overall processing time are achieved with only minimal degradation of physical properties. Heretofore it has been thought that a catalyst must be padded onto the fabric, either through an aqueous padding bath or by vapor padding, in order to achieve acceptable durable press properties and processing times. The present invention has achieved these goals without adding these catalysts to the system, thus avoiding sacrificing of significant losses in physical properties of the material.

**DESCRIPTION OF THE PREFERRED  
EMBODIMENTS**

50 The present invention is useful for treating various natural or artificial cellulosic fibers alone or in mixtures with each other in various proportions or as mixtures with other fibers. Such natural cellulosic fibers useful herein include, for example, cotton, linen, flax, hemp and jute. Useful regenerated or artificial cellulosic fibers include viscose rayon and cuprammonium rayon. Other fibers which may be used in blends with one or more of the above-mentioned cellulosic fibers are, for example, cellulose acetate, polyamides, polyesters, polyacrylonitrile, polyolefins, polyvinyl chloride, polyvinylidene chloride and polyvinyl alcohol fibers. Such blends preferably include at least about 15 percent by weight and most preferably at least about 35 percent by weight of cotton or other cellulosic fibers.

60 A fabric may be knit, woven or non-woven, or be any otherwise constructed fabric. The fabric may be flat,

creased, pleated, hemmed or sewn or otherwise formed to produce an article such as a garment of any desired shape prior or subsequent to contact with the reactive vapor phase containing formaldehyde. After processing, the formed cross-linked fabric will maintain substantially the original configuration for the life of the article, that is, a wash-wear or durable press fabric will be produced.

In accordance with the present invention, the cotton or cellulose-containing fabric is impregnated with a catalyst-free aqueous solution containing a monomeric compound which has at least one active hydrogen and reacts with formaldehyde, e.g., a compound of the amide type.

Suitable amide-type, reactive with formaldehyde compounds are typically water-soluble and include various ureas such as urea, butyl urea, ethylene urea, cyclic propylene urea, allyl urea, cyclic dihydroxyethylene urea, cyanuramide (melamine), thiourea as well as formamide, acetamide, maloamide, acrylamide, the lower alkyl (e.g., C<sub>1</sub> - C<sub>4</sub>) or hydroxyalkyl carbamates, such as ethyl carbamate and hydroxyl ethyl carbamate, aryl sulfonamides, such as benzene-sulfonamide or p-benzene-disulfonamide, the lower (e.g., C<sub>1</sub> - C<sub>4</sub>) alkyl sulfonamides or bis-sulfonamides such as methane-, ethane-, n-butane- or isobutane-sulfonamide, methylene-bis-methane-sulfonamide, ethylene-bis-methane-sulfonamide, 1,3-propane-bis-methane sulfonamide and so on. Urea and ethylene urea are preferred.

It is particularly advantageous to impregnate the fabric with the aqueous solution of the amide compound so as to produce a dry add-on of between about 0.5 and 25, preferably between about 2.5 and 15, percent by weight of the fabric.

The amide compound is preferably applied in an aqueous solution which may have a pH of from about 4 to 12. Generally, the aqueous solution will have an alkaline pH. Often, the pH will be between about 7 and less than about 11, preferably between about 8 and 9, and containing from about 1 to about 25 percent, preferably from about 3 to about 20 percent, most preferably from about 5 to about 15, percent of the amide.

Pretreatment of the fabric, prior to the exposure to the formaldehyde vapors, with polymeric resinous additives that form soft films such as conventional dispersions or latices, can result in unusually great incremental improvement in wrinkle recovery of the treated fabric. Polymer additives can also improve the flex, abrasion resistance and tear strength, or alter the ratio of dry wrinkle recovery to wet wrinkle recovery, or in some instances, shorten the reaction time needed to produce an acceptable durable press fabric. Polymeric additives suitable for such purposes are, in most cases, available commercially in concentrated aqueous latex forms, and it is desirable to dilute these to a concentration of about 1 to about 30, often from about 5 to about 15, percent polymer for padding onto the fabric. Suitable polymeric additives include solid resinous or rubbery acrylonitrile-butadiene copolymers and mixtures containing the same with various vinyl resins; polyethylene; deacetylated copolymers of ethylene and vinyl acetate; polyurethanes and various polymers of alkyl acrylates, and so forth, as is well-known in the art.

The impregnated fabric may be dried or conditioned to a moisture content of from about 2 up to about 100,

preferably from about 3 to about 65, most preferably from about 5 to about 15, percent by weight of the dry cellulosic fabric material.

If desired, the impregnated fabric may be dried and then used in garment manufacture (e.g., cutting, sewing and pressing) either immediately or after shipment to a different location or after storage of indefinite duration. The resulting garments may then be further treated as described hereinbelow either immediately or after storage of indefinite duration. The impregnated fabric (or garment) is exposed in the absence of a catalyst to an atmosphere containing formaldehyde vapors until a crease-proofing amount of an at least partially polymerized condensate of the monomeric compound and formaldehyde (e.g., a partially polymerized urea-formaldehyde condensate) in substantially water-insoluble form is affixed on the fabric without, however, effecting any substantial amount of cross-linking with the cellulosic fiber.

Although there is no substantial cross-linking, there apparently may be some binding, such as grafting of the condensate onto hydroxyl groups of the cellulose, taking place during the formaldehyde vapor contact step. A crease-proofing amount of the at least partially polymerized condensate is that amount which, when the fabric is post-heated, yields a fabric having acceptable durable press properties.

The atmosphere of the reaction zone may also contain air or any other non-acidic and non-deleterious gas which does not react with the formaldehyde or the monomeric compound and does not catalyze their reaction. Often, the reaction zone atmosphere contains from about 1 to about 100, preferably about 30 to about 95, volume percent formaldehyde.

Contact of the impregnated fabric with the formaldehyde vapor-containing atmosphere can be performed at a temperature of from about 100°C. to about 160°C., preferably from about 105°C. to about 120°C. for a time of from about 0.1 to about 60, preferably from about 0.5 to about 20, most preferably from about 1 to about 5 minutes.

Any suitable means to contact the fabric with the formaldehyde vapor-containing atmosphere may be employed. For example, a batch system utilizing a closed vessel or tube containing the reactive vapor phase atmosphere may be used into which the impregnated monomer-containing fabric may be placed and there exposed to the atmosphere for the appropriate time. In the alternative, a dynamic or continuous system can be used such as one wherein a gas stream containing formaldehyde vapor is passed through a closed elongated chamber through which the impregnated fabric or articles are also passed at an appropriate rate either concurrently or countercurrently relative to the gas. It is also possible to use combinations of the above, that is, such as by-passing a stream containing formaldehyde vapors over a stationary fabric.

The required formaldehyde vapor may be generated in any convenient manner, such as by heating a suspension of paraformaldehyde in mineral oil to generate formaldehyde gas which is then metered into the treating chamber. The formaldehyde vapor will be present in the reaction zone in an amount at least sufficient to react with all of the amide compound and generally will be present in an excess of that amount.

Typically, at the end of the formaldehyde vapor contacting step, the fabric is desirably heated at a tempera-

ture above about 80°C., e.g., in the range of from about 100°C. to about 180°C., preferably from about 140°C. to about 160°C. for from about 1 to about 20 minutes, preferably from about 3 to about 10 minutes, to further polymerize and cross-link the fabric thus improving its durability to laundering as well as improving the durable press characteristics of the treated fabric. In addition, this post-heating step will volatilize and remove any water vapor, unbound formaldehyde and other volatile residues. This post-heating step may also allow a reduction in the time of exposure to the formaldehyde vapor without sacrificing durable press performance. Heating the treating fabric may advantageously be performed in any suitable fabric heating chamber.

The treated fabric may be subjected to the post-heating step immediately after being exposed to the formaldehyde vapors or it may be stored for an indefinite period of time. If desired, the fabric may be used in garment manufacture after exposure to formaldehyde vapors and before the post-heating step. The treated fabric is preferably not washed prior to the post-heating step. Although we do not wish to be bound by theoretical considerations, it would appear that the least partially polymerized condensate formed in the formaldehyde vapor contact step may contain some reactive groups (such as methylol groups), the reactivity of which may be reduced by washing with water. The efficiency of the overall process is thus considerably reduced when the fabric is washed between these steps.

The invention is additionally illustrated in connection with the following examples which are to be considered as illustrative of the present invention. It should be understood, however, that the invention is not limited to the specific details of the examples.

### EXAMPLES

The reactor used in work was a cylindrical vessel having a capacity of about 71 liters constructed of one-eighth inch aluminum (42 cm. inside diameter and 57 cm. high). The walls of this reactor were heated with band heaters equipped with a 3-way switch which permits operation at 600, 1,200 or 2,400 watts. The reactor wall temperature was controlled by an adjustable bimetallic thermostat, and the reactor was surrounded by an insulating blanket. The gas content of the reactor was recirculated through an external recycle line by an aluminum pressure blower equipped with a heat slinger and high-temperature, lubricated sealed bearings. An adjustable damper in the recycle line permitted some control of the pressure within the reactor, but during normal operation, nearly atmospheric reactor pressure

was preferred.

Formaldehyde gas was conducted into the reactor through heated lines from a separate vessel where it was generated as needed by heating a suspension of between about 30 to 50 percent by weight (unless otherwise indicated) of paraformaldehyde in mineral oil. The reactor was further equipped with another line through which other gases such as air may be admitted when and as desired. The rate of flow of formaldehyde was controlled by regulating the temperature of the mineral oil between 100° and 140°C.

Unless otherwise indicated, all samples were tested wrinkle recovery angle in accordance with the test methods described in AATCC 66-1959T. For Elmerendorf Tearing Strength, test methods are in accordance with ASTM D-1424-59 and for Stoll Flex Abrasion Resistance, the test methods are in accordance with ASTM-D-61T (using head and tension loads of  $\frac{1}{2}$  and 2 pounds, respectively).

### EXAMPLE I

Samples of 100 percent cotton twill fabric (112  $\times$  50 thread) were padded with aqueous solutions containing from 0 to 20 percent urea and 10 percent (solids) urethane latex E-502 (Wyandotte Chemical Corporation) to give various add-ons. The impregnated samples were each dried to a moisture content of about 7 percent, exposed to a gaseous formaldehyde vapor atmosphere for 2 minutes at 120°C. and post-heated in air for 5 minutes at 150°C. Unless otherwise indicated, fabric samples in all of the examples were post-heated immediately after exposure to the gaseous formaldehyde atmosphere.

As shown in Table I, fabric properties were considerably improved when padded with a 1 percent urea-containing solution (about 2.6 percent monomer add-on calculated as the total add-on, Table I, minus the add-on value of polymeric additive for 0 percent urea, i.e., 4.1 weight percent) as compared with the 0 percent urea-containing solution. These improved properties were generally maintained or improved with each of the aqueous solutions having increased urea concentrations.

Table I indicates that as little as 1 percent urea in the aqueous solution imparts good durable press properties to cotton fabrics in the present process. These results are to be contrasted with conventional catalyzed durable press processes in which aqueous solution concentrations of 5 to 10 percent (solids) of the monomer or resin are necessary to achieve commercial levels of wrinkle recovery angles.

TABLE I

| Urea concentration in impregnating solution | Add-on, percent | Wrinkle recovery angle (degrees) |      |      |      | Tearing strength (Elmerendorf units) | Stoll flex abrasion warp (cycles) | Tensile properties        |                             |                         |                           |                             |                         |            |  |
|---------------------------------------------|-----------------|----------------------------------|------|------|------|--------------------------------------|-----------------------------------|---------------------------|-----------------------------|-------------------------|---------------------------|-----------------------------|-------------------------|------------|--|
|                                             |                 | Dry                              |      | Wet  |      |                                      |                                   | Warp                      |                             |                         | Fill                      |                             |                         |            |  |
|                                             |                 | Warp                             | Fill | Warp | Fill |                                      |                                   | Work-to-rupture (in.-lb.) | Extension at break, percent | Breaking strength (lb.) | Work-to-rupture (in.-lb.) | Extension at break, percent | Breaking strength (lb.) |            |  |
| 0-----                                      | 4.1             | 119                              | 108  | 136  | 122  | 164.8                                | 108.8                             | 933                       | 35.6                        | 18.9                    | 180.5                     | 12.3                        | 19.4                    | 71.3 ----- |  |
| 1-----                                      | 6.7             | 146                              | 129  | 157  | 142  | 218.0                                | 116.0                             | 1,175                     | 18.1                        | 13.9                    | 125.5                     | 6.6                         | 14.4                    | 48.6 5.1   |  |
| 2.5-----                                    | 6.8             | 150                              | 140  | 150  | 144  | 212.5                                | 122.5                             | 1,338                     | 18.2                        | 13.6                    | 125.0                     | 6.5                         | 14.2                    | 50.0 5.0   |  |
| 5.0-----                                    | 7.4             | 152                              | 132  | 155  | 138  | 237.5                                | 127.0                             | 1,310                     | 20.1                        | 14.6                    | 137.0                     | 6.7                         | 14.5                    | 52.3 5.0   |  |
| 7.5-----                                    | 8.1             | 155                              | 136  | 156  | 144  | 213.5                                | 124.2                             | 1,462                     | 22.2                        | 14.2                    | 144.0                     | 6.1                         | 15.2                    | 47.4 5.2   |  |
| 10.0-----                                   | 10.2            | 152                              | 136  | 152  | 142  | 201.0                                | 112.0                             | 1,465                     | 19.6                        | 13.4                    | 133.5                     | 6.3                         | 15.1                    | 49.5 5.3   |  |
| 15.0-----                                   | 19.5            | 154                              | 148  | 169  | 154  | 129.0                                | 84.8                              | 626                       | 15.6                        | 9.8                     | 137.0                     | 4.8                         | 12.6                    | 48.3 5.4   |  |
| 20.0-----                                   | 23.9            | 147                              | 144  | 166  | 149  | 134.3                                | 83.2                              | 754                       | 19.4                        | 10.7                    | 155.5                     | 7.2                         | 13.9                    | 59.7 5.6   |  |
| N.a.-----                                   | N.a.            | 74                               | 75   | 73   | 81   | 169.4                                | 98.3                              | 421                       | 31.8                        | 13.2                    | 187.0                     | 11.8                        | 17.9                    | 71.6 ----- |  |

\*Untreated control.

## EXAMPLE II

The effect of formaldehyde exposure time and the presence of steam on fabric properties was studied in this Example in which samples of the fabric of Example I were impregnated with an aqueous solution containing 10 percent urea and 10 percent (solids) urethane latex E-502, exposed to formaldehyde vapor for from 1 to 4 minutes at 120°C. in the presence or absence of any steam and then post-heated for 5 minutes at 150°C. The resulting fabric properties shown in Table II indicate that small increases in wrinkle recovery angle and corresponding decreases in tensile strength were obtained as exposure time was increased from 1 to 4 minutes.

material upon which the resin is deposited.

The effect of post-heating temperature is shown in Table III-B. Although the amount of amide add-on increased with increased temperature, most other properties did not. After 10 laundering cycles, the fabric properties showed little change, indicating that the process of this invention can be operated within wide ranges of post-heating time and temperature without significantly affecting the balance of fabric properties.

It is known that gaseous formaldehyde generated by heating paraformaldehyde-mineral oil slurries may contain a minor amount (i.e., less than 5 weight percent) of impurities such as water, methanol, methyl formate and formic acid. Formic acid is a known catalyst

TABLE II

| HCHO<br>exposure<br>time at<br>120°<br>C. (min.) | HCHO<br>steam<br>exposure<br>time at<br>120° C.<br>(min.) | Add-<br>on,<br>per-<br>cent | Wrinkle recovery angle<br>(degrees) |      |      |      | Tearing<br>strength<br>(Elmendorf<br>units) |      | Tensile properties                                    |                                      |                                        |                               |                                      |                                        |                               |
|--------------------------------------------------|-----------------------------------------------------------|-----------------------------|-------------------------------------|------|------|------|---------------------------------------------|------|-------------------------------------------------------|--------------------------------------|----------------------------------------|-------------------------------|--------------------------------------|----------------------------------------|-------------------------------|
|                                                  |                                                           |                             | Dry                                 |      | Wet  |      | Warp                                        |      | Warp                                                  |                                      | Fill                                   |                               |                                      |                                        |                               |
|                                                  |                                                           |                             | Warp                                | Fill | Warp | Fill | Warp                                        | Fill | Stoll<br>flex<br>abrasion<br>work<br>wrap<br>(cycles) | Work-<br>to-<br>rupture<br>(in.-lb.) | Extens-<br>ion at<br>break,<br>percent | Breaking<br>strength<br>(lb.) | Work-<br>to-<br>rupture<br>(in.-lb.) | Extens-<br>ion at<br>break,<br>percent | Breaking<br>strength<br>(lb.) |
| 1.                                               | 0                                                         | 11.8                        | 150                                 | 180  | 147  | 142  | 162.7                                       | 98.8 | 1,234                                                 | 19.6                                 | 11.5                                   | 147.5                         | 6.2                                  | 14.8                                   | 51.0                          |
| 2.                                               | 0                                                         | 13.7                        | 154                                 | 142  | 156  | 146  | 157.5                                       | 90.0 | 1,036                                                 | 17.3                                 | 11.0                                   | 137.0                         | 5.8                                  | 13.4                                   | 49.9                          |
| 3.                                               | 0                                                         | 13.9                        | 160                                 | 147  | 160  | 148  | 154.0                                       | 89.8 | 902                                                   | 17.6                                 | 11.4                                   | 138.5                         | 5.9                                  | 14.2                                   | 49.6                          |
| 4.                                               | 0                                                         | 15.0                        | 165                                 | 148  | 160  | 150  | 138.0                                       | 87.0 | 854                                                   | 14.5                                 | 10.4                                   | 127.0                         | 4.8                                  | 13.0                                   | 47.0                          |
| 0.                                               | 1                                                         | 13.0                        | 152                                 | 142  | 158  | 145  | 146.8                                       | 86.0 | 950                                                   | 17.3                                 | 11.0                                   | 137.5                         | 5.2                                  | 14.6                                   | 44.6                          |
| 0.                                               | 2                                                         | 14.6                        | 152                                 | 146  | 154  | 152  | 148.5                                       | 87.5 | 811                                                   | 15.8                                 | 10.8                                   | 131.0                         | 5.3                                  | 14.0                                   | 48.0                          |
| 0.                                               | 3                                                         | 15.1                        | 159                                 | 146  | 155  | 150  | 138.5                                       | 79.5 | 790                                                   | 14.9                                 | 10.3                                   | 129.0                         | 4.5                                  | 12.7                                   | 43.9                          |
| 0.                                               | 4                                                         | 14.3                        | 160                                 | 154  | 154  | 155  | 138.0                                       | 89.8 | 825                                                   | 15.9                                 | 10.4                                   | 130.0                         | 4.9                                  | 13.9                                   | 43.6                          |
| N.a.*                                            | N.a.                                                      | N.a.                        | 74                                  | 75   | 73   | 81   | 169.4                                       | 9.3  | 421                                                   | 31.8                                 | 13.2                                   | 187.0                         | 11.8                                 | 17.9                                   | 71.6                          |

\*Untreated control.

## EXAMPLE III

Samples of the fabric of Example I which were impregnated with solutions containing 10 percent urea and 10 percent (solids) urethane latex E-502, dried to a moisture content of about 7 percent and exposed to formaldehyde vapor for 2 minutes at 120°C., were post-heated at varying temperatures and times. The data as shown in Table III-A indicates that although the tensile strength remains essentially unchanged, the dry and wet wrinkle recovery angles were substantially increased in the post-heated sample as compared with a sample which was not post-heated.

Thus, although the theoretical mechanism is not clear, it appears that further condensation probably occurs between urea and formaldehyde during the post-heating step and also that further bonds may be formed between the urea-formaldehyde resin and the cellulosic

for use in catalytically effective amounts in durable press processes using formaldehyde. However, the small amount of formic acid which could (depending upon the gas purity) be present in the process of the present invention is so small as to be insufficient to cause any significant change in the balance of properties obtained as compared with those obtained when carrying out the reaction in the absence of any catalytic material. That is, the small amount of formic acid or other material normally considered a catalyst in a durable press process including formaldehyde which could be present in the process of the present invention is less than a catalytically effective amount and so small as to be insufficient to cause any significant change in the balance of properties obtained as compared with those obtained when carrying out the reaction in the absence of any amount of a material normally considered a catalyst.

TABLE III-A

| Post heating<br>time at<br>150° C.<br>(min.) | Number<br>of<br>washings | Add-<br>on,<br>per-<br>cent | Wrinkle Recovery Angle<br>(degrees) |      |      |      | Tearing<br>strength<br>(Elmendorf<br>units) |       | Tensile properties                                    |                                      |                                        |                               |                                      |                                        |                               |      |
|----------------------------------------------|--------------------------|-----------------------------|-------------------------------------|------|------|------|---------------------------------------------|-------|-------------------------------------------------------|--------------------------------------|----------------------------------------|-------------------------------|--------------------------------------|----------------------------------------|-------------------------------|------|
|                                              |                          |                             | Dry                                 |      | Wet  |      | Warp                                        |       | Warp                                                  |                                      | Fill                                   |                               |                                      |                                        |                               |      |
|                                              |                          |                             | Warp                                | Fill | Warp | Fill | Warp                                        | Fill  | Stoll<br>flex<br>abrasion<br>work<br>wrap<br>(cycles) | Work-<br>to-<br>rupture<br>(in.-lb.) | Extens-<br>ion at<br>break,<br>percent | Breaking<br>strength<br>(lb.) | Work-<br>to-<br>rupture<br>(in.-lb.) | Extens-<br>ion at<br>break,<br>percent | Breaking<br>strength<br>(lb.) |      |
| 0.                                           | 1                        | 8.9                         | 136                                 | 117  | 141  | 137  | 265.0                                       | 153.5 | 888                                                   | 28.0                                 | 16.0                                   | 153.5                         | 8.6                                  | 16.4                                   | 54.6                          |      |
| 1.                                           | 1                        | 11.6                        | 146                                 | 122  | 162  | 146  | 199.5                                       | 126.8 | 1,084                                                 | 21.0                                 | 13.4                                   | 138.5                         | 7.3                                  | 15.6                                   | 53.1                          |      |
| 2.                                           | 1                        | 11.9                        | 148                                 | 134  | 158  | 151  | 199.3                                       | 116.8 | 1,608                                                 | 23.2                                 | 13.4                                   | 151.0                         | 7.3                                  | 16.2                                   | 53.6                          |      |
| 3.                                           | 1                        | 12.9                        | 152                                 | 138  | 162  | 149  | 178.0                                       | 115.8 | 1,428                                                 | 21.4                                 | 13.0                                   | 147.0                         | 7.2                                  | 15.2                                   | 53.4                          |      |
| 4.                                           | 1                        | 13.9                        | 156                                 | 140  | 160  | 151  | 152.0                                       | 97.5  | 1,161                                                 | 17.7                                 | 11.4                                   | 136.0                         | 6.1                                  | 14.8                                   | 50.2                          |      |
| 5.                                           | 1                        | 13.3                        | 156                                 | 150  | 158  | 157  | 159.8                                       | 95.5  | 1,080                                                 | 19.3                                 | 11.8                                   | 142.0                         | 5.3                                  | 13.8                                   | 47.2                          |      |
| 0.                                           | 10                       | 8.0                         | 138                                 | 122  | 142  | 142  | 130                                         | 265.0 | 143.5                                                 | 658                                  | 23.9                                   | 15.5                          | 141.5                                | 8.4                                    | 15.4                          | 57.2 |
| 1.                                           | 10                       | 9.1                         | 140                                 | 122  | 150  | 136  | 210.5                                       | 131.2 | 732                                                   | 21.4                                 | 14.0                                   | 140.5                         | 7.8                                  | 15.5                                   | 55.4                          |      |
| 2.                                           | 10                       | 9.9                         | 148                                 | 133  | 151  | 142  | 193.5                                       | 124.5 | 1,214                                                 | 20.9                                 | 13.8                                   | 141.5                         | 7.5                                  | 15.2                                   | 56.0                          |      |
| 3.                                           | 10                       | 10.0                        | 150                                 | 134  | 149  | 142  | 202.5                                       | 120.2 | 1,210                                                 | 20.9                                 | 13.2                                   | 142.5                         | 7.8                                  | 15.4                                   | 56.0                          |      |
| 4.                                           | 10                       | 11.8                        | 154                                 | 136  | 157  | 144  | 161.0                                       | 100.2 | 1,275                                                 | 17.3                                 | 12.2                                   | 133.0                         | 5.2                                  | 14.4                                   | 45.0                          |      |
| 5.                                           | 10                       | 11.7                        | 152                                 | 145  | 158  | 149  | 166.8                                       | 113.5 | 1,169                                                 | 18.3                                 | 12.4                                   | 134.0                         | 5.9                                  | 14.0                                   | 49.7                          |      |
| N.a.*                                        | N.a.                     | N.a.                        | 74                                  | 75   | 73   | 81   | 169.4                                       | 98.3  | 421                                                   | 31.8                                 | 13.2                                   | 187.0                         | 11.8                                 | 17.9                                   | 71.6                          |      |

\*Untreated control.

TABLE III-B

| Post-heating<br>temp. (°C.) | Number<br>of<br>washings | Add-<br>on,<br>per-<br>cent | Tensile properties                  |     |     |     |                                          |       |       |      |                                                    |                                           |                                           |                               |      |      |
|-----------------------------|--------------------------|-----------------------------|-------------------------------------|-----|-----|-----|------------------------------------------|-------|-------|------|----------------------------------------------------|-------------------------------------------|-------------------------------------------|-------------------------------|------|------|
|                             |                          |                             | Wrinkle Recovery Angle<br>(degrees) |     |     |     | Tearing strength<br>(Elmendorf<br>units) |       |       |      | Warp                                               |                                           |                                           |                               |      |      |
|                             |                          |                             | Dry                                 |     | Wet |     | Warp                                     | Fill  | Warp  | Fill | Stoll<br>flex<br>abra-<br>sion<br>wrap<br>(cycles) | Work-<br>to-<br>rup-<br>ture<br>(in.-lb.) | Extен-<br>sion<br>at<br>break,<br>percent | Breaking<br>strength<br>(lb.) |      |      |
| 100                         | 1                        | 11.6                        | 143                                 | 136 | 150 | 148 | 177.0                                    | 113.0 |       |      | 18.6                                               | 13.4                                      | 132.0                                     | 7.3                           | 15.3 | 53.2 |
| 120                         | 1                        | 11.5                        | 153                                 | 140 | 154 | 147 | 163.7                                    | 101.0 |       |      | 18.5                                               | 12.4                                      | 136.5                                     | 6.5                           | 14.4 | 51.7 |
| 140                         | 1                        | 12.7                        | 158                                 | 141 | 154 | 152 | 145.7                                    | 92.8  | 979   |      | 17.4                                               | 11.6                                      | 136.0                                     | 5.5                           | 13.2 | 49.2 |
| 160                         | 1                        | 13.1                        | 159                                 | 148 | 153 | 156 | 134.8                                    | 86.8  | 890   |      | 16.7                                               | 11.0                                      | 137.0                                     | 5.4                           | 13.2 | 48.5 |
| 100                         | 10                       | 11.6                        | 142                                 | 122 | 149 | 142 | 173.0                                    | 117.5 |       |      | 21.3                                               | 14.8                                      | 139.5                                     | 6.7                           | 15.7 | 51.3 |
| 120                         | 10                       | 11.6                        | 152                                 | 134 | 158 | 146 | 151.2                                    | 97.0  |       |      | 19.1                                               | 11.0                                      | 141.0                                     | 6.9                           | 15.4 | 53.2 |
| 140                         | 10                       | 12.4                        | 150                                 | 134 | 153 | 146 | 152.8                                    | 92.2  | 874   |      | 17.8                                               | 12.4                                      | 136.5                                     | 5.4                           | 13.6 | 48.0 |
| 160                         | 10                       | 12.6                        | 155                                 | 138 | 153 | 149 | 150.0                                    | 92.0  | 1,006 |      | 17.2                                               | 11.8                                      | 136.0                                     | 5.5                           | 13.4 | 50.0 |
| N.a.*                       | N.a.                     | N.a.                        | 74                                  | 75  | 73  | 81  | 169.4                                    | 98.3  | 421   |      | 31.8                                               | 13.2                                      | 187.0                                     | 11.8                          | 17.0 | 71.6 |

\*Untreated control.

## EXAMPLE IV

The effects of the moisture content of the cotton fabric prior to formaldehyde treatment were studied. Samples of the cotton twill fabric of Example I were padded with a solution containing 10 percent urea and 10 percent (solids) urethane latex E-502, dried and conditioned to various levels of moisture content, exposed to formaldehyde vapor for 2 minutes at 120°C. and then post-heated for 5 minutes at 150°C.

It is known that in at least some prior art catalytic processes increasing the moisture content of cotton fabrics prior to treatment with formaldehyde vapors increases the amount of absorbed formaldehyde as well as the amount of fixed formaldehyde. In the present process, however, the amount of water in cotton fibers does not appear to be a critical parameter in determining the extent of reaction between formaldehyde and urea. As shown in Table IV, add-ons for all samples were approximately equal and all fabric samples had acceptable durable press properties.

The effect of surface polymeric additives on wrinkle recovery angle and strength loss was studied by impregnating samples of the fabric of Example I with aqueous solutions of various commercially available polymeric additives with and without urea also being present in the aqueous solutions. The impregnated fabric samples were each dried at 80°C. to a moisture content of about 7 percent, exposed to formaldehyde vapor for 2 minutes at 120°C. and post-heated for 5 minutes at 150°C. Results are shown in Table V. As expected, fabrics impregnated with the stronger (higher film modulus value) polymeric additives such as Rhoplex K-87 and urethane latex P-501 generally show greater strength and lower wrinkle recovery angles than the fabrics impregnated with the lower strength polymeric additives Rhoplex K-14 and urethane latex E-502.

## EXAMPLE V

The effect of time and/or washing between exposure

TABLE IV

| Add-on,<br>percent | Initial<br>moisture<br>content,<br>percent | No.<br>of<br>wash-<br>ings | Wrinkle recovery angle<br>(degrees) |     |      |      | Tearing<br>strength<br>(Elmendorf<br>units) | Stoll<br>flex<br>abra-<br>sion<br>wrap<br>(cycles) | Warp  |      |                                           |                                           | Fill                          |                                           |                                           |                               |
|--------------------|--------------------------------------------|----------------------------|-------------------------------------|-----|------|------|---------------------------------------------|----------------------------------------------------|-------|------|-------------------------------------------|-------------------------------------------|-------------------------------|-------------------------------------------|-------------------------------------------|-------------------------------|
|                    |                                            |                            | Dry                                 |     | Wet  |      |                                             |                                                    | Warp  | Fill | Work-<br>to-<br>rup-<br>ture<br>(in.-lb.) | Extен-<br>sion<br>at<br>break,<br>percent | Breaking<br>strength<br>(lb.) | Work-<br>to-<br>rup-<br>ture<br>(in.-lb.) | Extен-<br>sion<br>at<br>break,<br>percent | Breaking<br>strength<br>(lb.) |
|                    |                                            |                            |                                     |     | Warp | Fill |                                             |                                                    |       |      |                                           |                                           |                               |                                           |                                           |                               |
| 11.3               | 3.5                                        | 1                          | 150                                 | 132 | 152  | 144  | 179.0                                       | 141.2                                              | 1,886 | 24.0 | 14.8                                      | 145.5                                     | 8.2                           | 15.6                                      | 51.6                                      |                               |
| 11.4               | 7.2                                        | 1                          | 161                                 | 150 | 159  | 156  | 139.8                                       | 87.5                                               | 932   | 15.2 | 10.6                                      | 129.5                                     | 5.4                           | 13.5                                      | 47.2                                      |                               |
| 11.8               | 16.0                                       | 1                          | 158                                 | 152 | 167  | 153  | 135.2                                       | 84.0                                               | 847   | 16.2 | 11.0                                      | 131.5                                     | 5.8                           | 13.8                                      | 50.9                                      |                               |
| 11.4               | 3.5                                        | 10                         | 140                                 | 125 | 158  | 158  | 202.0                                       | 158.2                                              | 1,866 | 27.9 | 17.5                                      | 148.0                                     | 8.6                           | 16.4                                      | 57.7                                      |                               |
| 11.2               | 7.2                                        | 10                         | 158                                 | 142 | 164  | 152  | 163.2                                       | 99.8                                               | 1,258 | 17.7 | 12.1                                      | 131.0                                     | 5.5                           | 14.0                                      | 46.0                                      |                               |
| 11.7               | 16.0                                       | 10                         | 154                                 | 140 | 169  | 155  | 157.0                                       | 88.5                                               | 1,222 | 16.3 | 11.8                                      | 128.0                                     | 5.4                           | 14.0                                      | 46.1                                      |                               |
| N.a.*              | N.a.                                       | N.a.                       | 74                                  | 75  | 73   | 81   | 169.4                                       | 98.3                                               | 421   | 31.8 | 13.2                                      | 187.0                                     | 11.8                          | 17.9                                      | 71.6                                      |                               |

\*Untreated control.

TABLE V

| Additive<br>(% solids)         | Add-on<br>(%)         | Wrinkle Recovery<br>Angle, W + F<br>(degrees) |                       | Tensile Strength<br>(% retention) |                     |  |  |
|--------------------------------|-----------------------|-----------------------------------------------|-----------------------|-----------------------------------|---------------------|--|--|
|                                |                       | Dry                                           | Wet                   | Warp                              | Fill                |  |  |
| 2.5% Rhoplex K-87 <sup>a</sup> | 1.8(8.3) <sup>a</sup> | 170(296) <sup>a</sup>                         | 195(292) <sup>a</sup> | 90(74) <sup>a</sup>               | 97(66) <sup>a</sup> |  |  |
| 5.0% Rhoplex K-87              | 3.1(9.7)              | 177(296)                                      | 204(300)              | 89(74)                            | 108(71)             |  |  |
| 7.5% Rhoplex K-87              | 4.1(11.1)             | 191(294)                                      | 206(303)              | 91(73)                            | 100(70)             |  |  |
| 10.0% Rhoplex K-87             | 5.4(12.8)             | 190(300)                                      | 217(301)              | 94(78)                            | 95(77)              |  |  |
| 2.5% Rhoplex K-14 <sup>b</sup> | 1.0(7.6)              | 191(265)                                      | 188(258)              | 79(71)                            | 91(68)              |  |  |
| 5.0% Rhoplex K-14              | 2.5(8.6)              | 206(280)                                      | 218(261)              | 74(73)                            | 83(68)              |  |  |

TABLE V - Continued

| Additive<br>(% solids)        | Add-on<br>(%) | Wrinkle Recovery<br>Angle, W + F<br>(degrees) |          | Tensile Strength<br>(% retention) |         |
|-------------------------------|---------------|-----------------------------------------------|----------|-----------------------------------|---------|
|                               |               | Dry                                           | Wet      | Warp                              | Fill    |
| 7.5% Rhoplex K-14             | 2.9(9.4)      | 222(280)                                      | 217(283) | 75(68)                            | 83(59)  |
| 10.0% Rhoplex K-14            | 4.3(11.6)     | 225(274)                                      | 235(279) | 77(69)                            | 79(66)  |
| 2.5% U. L. P-501 <sup>c</sup> | 0.9(8.3)      | 184(284)                                      | 204(274) | 94(74)                            | 101(74) |
| 5.0% U. L. P-501              | 2.4(10.2)     | 205(288)                                      | 224(281) | 94(81)                            | 101(75) |
| 7.5% U. L. P-501              | 3.8(12.0)     | 204(293)                                      | 238(296) | 98(82)                            | 98(81)  |
| 10.0% U. L. P-501             | 5.0(13.4)     | 222(288)                                      | 254(298) | 96(85)                            | 98(78)  |
| 2.5% U. L. E-502 <sup>d</sup> | 2.1(6.4)      | 206(268)                                      | 222(264) | 89(72)                            | 93(76)  |
| 5.0% U. L. E-502              | 3.2(8.4)      | 214(285)                                      | 232(286) | 78(77)                            | 89(66)  |
| 7.5% U. L. E-502              | 4.4(10.3)     | 235(298)                                      | 259(293) | 81(72)                            | 94(66)  |
| 10.0% U. L. E-502             | 5.2(12.5)     | 227(302)                                      | 263(305) | 82(71)                            | 89(69)  |
| Control                       | n.a.          | 149                                           | 154      | 100                               | 100     |

a—an acrylic resin available from the Rohm and Haas Co.

b—an acrylic emulsion available from the Rohm and Haas Co.

c-Urethane Latex P-501 available from the Wyandotte Chemical Corp.

d-Urethane Latex E-502 available from the Wyandotte Chemical Corp.

e-Figures in parenthesis denote values for fabric treated in the presence of urea (10% based on the weight of pad bath).

to the foamaldehyde vapor and the post-heating step were considered in this example.

Samples of the fabric of Example I were padded with an aqueous solution containing 10 weight percent urea and 10 weight percent urethane latex E-502. The impregnated samples were dried to a moisture content of about 7 percent, pressed and exposed to a 100 percent

Angles and Durable Press Ratings as compared with the untreated control, both show unacceptable properties for commercial durable press materials. Both samples also show properties substantially less than the samples of Table VI-A. In addition, this data shows that post-heating only moderately improves the durable press properties of a washed sample.

TABLE VI-A

| Time between exposure to gaseous formaldehyde and post-heating, hours | Wrinkle Recovery Angles, (W + F) Durable Press Ratings, degrees |     |     |
|-----------------------------------------------------------------------|-----------------------------------------------------------------|-----|-----|
|                                                                       | Dry                                                             | Wet |     |
| 0                                                                     | 292                                                             | 297 | 4.1 |
| 1                                                                     | 293                                                             | 310 | 4.1 |
| 2                                                                     | 288                                                             | 314 | 4.1 |
| 4                                                                     | 286                                                             | 327 | 4.1 |
| 6                                                                     | 285                                                             | 301 | 4.0 |
| 24                                                                    | 274                                                             | 316 | 4.0 |
| 72                                                                    | 309                                                             | 315 | 4.0 |
| 144                                                                   | 299                                                             | 330 | 4.0 |
| Untreated Control                                                     | 149                                                             | 154 | 1.5 |

formaldehyde vapor atmosphere for 2 minutes at 120°C. The samples were held for varying times and then post-heated in air at 150°C. for 5 minutes. The results are shown in Table VI-A.

The results obtained indicate that the impregnated fabrics were not affected by delaying the post-heating step since the resulting properties were essentially the same (and within the limits of experimental error) whether the fabric was post-heated immediately or after 6 days.

Samples of the same fabrics as above were impregnated, dried and exposed to gaseous formaldehyde in the same manner as above and were washed immediately after exposure to the formaldehyde vapors. Sample I was not post-heated. Sample II was post-heated for 5 minutes at 150°C. and washed again.

The results obtained are shown in Table VI-B. Although both samples show higher Wrinkle Recovery

TABLE VI-B

| Sample            | Wrinkle Recovery Angle (W + F), Degrees | Durable Press Ratings, Wet |
|-------------------|-----------------------------------------|----------------------------|
| Dry               |                                         |                            |
| I                 | 230                                     | 3.1                        |
| II                | 245                                     | 3.2                        |
| Untreated Control | 149                                     | 1.5                        |

#### EXAMPLE VII

The interaction of the impregnation of the amide, impregnation of the polymeric additive and contact with gaseous formaldehyde was considered in this example. The varying treatments applied to the fabric samples as well as the results obtained are shown in Table VII.

TABLE VII

| Pretreatment                         | Posttreatment          | Formaldehyde Exposure Time <sup>a</sup> (min) | Wrinkle Recovery |                 | Tensile Strength (% retention) |
|--------------------------------------|------------------------|-----------------------------------------------|------------------|-----------------|--------------------------------|
|                                      |                        |                                               | Dry              | Angle (degrees) |                                |
| None                                 | None                   | 1                                             | 145              | 172             | 97                             |
|                                      |                        | 5                                             | 142              | 164             | 88                             |
|                                      |                        | 10                                            | 133              | 166             | 86                             |
|                                      |                        | 15                                            | 142              | 164             | 99                             |
|                                      |                        | 20                                            | 143              | 170             | 95                             |
| 10% E-502 <sup>b</sup>               | None                   | 0                                             | 190              | 167             | 88                             |
|                                      |                        | 1                                             | 236              | 260             | 85                             |
|                                      |                        | 5                                             | 235              | 259             | 89                             |
|                                      |                        | 10                                            | 246              | 266             | 86                             |
|                                      |                        | 15                                            | 263              | 284             | 83                             |
|                                      |                        | 20                                            | 252              | 280             | 82                             |
| 10% Urea                             | None                   | 1                                             | 267              | 253             | 65                             |
|                                      |                        | 2                                             | 262              | 248             | 70                             |
|                                      |                        | 3                                             | 251              | 243             | 72                             |
|                                      |                        | 4                                             | 270              | 250             | 76                             |
| 10% Urea                             | 10% E-502 <sup>b</sup> | 1                                             | 298              | 285             | 50                             |
|                                      |                        | 2                                             | 288              | 277             | 67                             |
|                                      |                        | 3                                             | 291              | 279             | 69                             |
|                                      |                        | 4                                             | 294              | 280             | 62                             |
| 10% Urea +<br>10% E-502 <sup>b</sup> | None                   | 1                                             | 280              | 289             | 71                             |
|                                      |                        | 2                                             | 296              | 302             | 70                             |
|                                      |                        | 3                                             | 307              | 308             | 69                             |
|                                      |                        | 4                                             | 303              | 310             | 66                             |

<sup>a</sup> All fabrics postheated for 5 min at 150°C.<sup>b</sup> Percent solids in aqueous solutions

As shown therein, samples of the fabric of Example I exposed to gaseous formaldehyde for 1 to 20 minutes at 120°C. without prior impregnation with the monomer or the surface polymeric additive exhibited no increases in wrinkle recovery angles (hereinafter WRAs) even after 20 minutes of treatment. These fabrics, however, suffered tensile strength losses of 1 to 14 percent respectively.

Fabrics padded with an aqueous solution containing 10 percent (solids) urethane latex E-502 exposed to formaldehyde vapor for 5 to 20 minutes and post-heated for 5 minutes at 150°C., exhibited moderate degrees of recovery angles (235° – 263° dry and 259° – 280° wet), probably indicating a chemical interaction between the urethane latex, formaldehyde and cellulose. Although the dry WRA's proved to be nondurable to laundering, the wet WRA's were unchanged after 10 laundering cycles. The loss in tensile strength exhibited by these samples was between 11 and 18 percent.

In another part of the experiment, fabrics were padded with a 10 percent urea solution, dried to a moisture content of about 7 percent, exposed to gaseous formaldehyde for 1 to 4 minutes at 120°C., and post-heated for 5 minutes at 150°C. These fabrics also showed only moderate WRA's but higher strength losses in fabrics treated with formaldehyde in the presence of the urethane latex alone.

To study the effect of applying the urethane latex to fabrics that had been treated with the urea formaldehyde system in the absence of a polymeric additive, fabrics from the previous experiment were re-padded with an aqueous solution containing 10 percent solid urethane latex E-502, dried and then cured for 5 minutes at 150°C. As shown in Table VIII, the dry and wet WRA's increased by about 30° each while the tensile strengths decreased 3 to 10 percent. After 10 laundering cycles, most properties showed little change.

The principles, preferred embodiments and modes of operation of the present invention have been described in the foregoing specification. The invention which is intended to be protected herein, however, is not to be

construed as limited to the particular forms disclosed, since these are to be regarded as illustrative rather than restrictive. Variations and changes may be made by those skilled in the art without departing from the spirit of the invention.

What is claimed is:

1. A non-catalytic process for improving the dimensional stability, wrinkle resistance, smooth drying characteristics and total shape retentivity of a cellulose fiber-containing fabric which comprises:

a. applying to a cellulose fiber-containing fabric a catalyst-free aqueous solution of a monomeric amide compound which has at least one active hydrogen and reacts with formaldehyde;

b. exposing the impregnated fabric to an atmosphere containing formaldehyde vapors in the essential absence of an acidic catalyst until a crease-proofing amount of an at least partially polymerized condensate of the monomeric amide compound and formaldehyde in substantially water in soluble form is affixed on said fabric without effecting any substantial amount of cross-linking with the cellulose fiber; and

c. post-heating said fabric in an inert gaseous atmosphere in the essential absence of an acidic catalyst at a temperature of from about 100°C. to about 180°C. for from about 1 to about 20 minutes to further polymerize and cross-link the fabric.

2. The process of claim 1 wherein said amide is urea and further wherein said fabric is impregnated with the aqueous solution of urea so as to produce a dry add-on of between about 0.5 and 25 percent by weight of the fabric.

3. The process of claim 1 wherein said impregnated fabric is formed into a garment prior to exposure to the formaldehyde vapors.

4. The process of claim 1 wherein said impregnated fabric is dried to a moisture content of from about 2 to about 100 percent by weight of the dry cellulosic fabric material prior to exposure to the formaldehyde vapor-containing atmosphere.

5. A non-catalytic process for improving the dimensional stability, wrinkle resistance, smooth drying char-

acteristics and total shape retentivity of a cellulose fiber-containing fabric which comprises:

- a. applying to a cellulose fiber-containing fabric a catalyst-free aqueous solution of a monomeric amide compound which has at least one active hydrogen and reacts with formaldehyde and a polymeric film-forming additive so as to produce an impregnated fabric having a dry add-on of between about 0.5 and 25 percent by weight of the fabric of the said monomeric amide compound;
- b. drying said impregnated fabric;
- c. forming said impregnated fabric into a garment;
- d. exposing the impregnated garment to an atmosphere containing formaldehyde vapors in the essential absence of an acidic catalyst at a temperature of from about 100°C. to about 160°C. for from about 0.1 to about 60 minutes until a crease-proofing amount of an at least partially polymerized condensate of the monomeric amide compound and formaldehyde in substantially water-insoluble form is affixed on said fabric without effecting any substantial amount of cross-linking with the cellulose fiber;
- e. post-heating said exposed garment in an inert gaseous atmosphere in the essential absence of an acidic catalyst at a temperature of from about 100°C. to about 180°C. for from about 1 to about 20 minutes to further polymerize and cross-link the fabric.

6. The non-catalytic process of claim 5 wherein said amide is urea.

7. The non-catalytic process of claim 6 wherein said impregnated fabric is dried to a moisture content of from about 3 to about 65 percent by weight of the dry cellulose fiber-containing fabric prior to exposure to

5

10

20

25

30

40

45

50

55

60

65

the formaldehyde vapor-containing atmosphere.

8. The non-catalytic process of claim 7 wherein said impregnated fabric is exposed to the formaldehyde vapors for a time of from about 0.5 to about 20 minutes.

9. A non-catalytic process for improving the dimensional stability, wrinkle resistance, smooth drying characteristics and total shape retentivity of a cellulose fiber-containing fabric which consists essentially of the following sequential steps:

- a. applying to the cellulose fiber-containing fabric a catalyst-free aqueous solution containing from about 5 to about 15 percent by weight of the solution of urea and from about 5 to about 15 percent of a film-forming polymeric additive;
- b. drying the impregnated fabric to a moisture content of from about 5 to about 15 percent by weight of the dry cellulose fiber-containing fabric;
- c. exposing the dried, impregnated fabric to a vapor phase atmosphere consisting essentially of formaldehyde vapors in an uncatalyzed reaction zone maintained at a temperature of from about 105°C. to about 120°C. for a time of from about 1 to about 5 minutes, until a crease-proofing amount of an at least partially polymerized amide-formaldehyde condensate in substantially water-insoluble form is affixed on said fabric without any substantial cross-linking with the cellulose fiber; and
- d. immediately thereafter post-heating said fabric in an inert gaseous atmosphere in the essential absence of an acidic catalyst at a temperature of from about 140°C. to about 160°C. for a time of from about 3 to about 10 minutes to further polymerize and cross-link said fabric.

\* \* \* \* \*